

## UNITED STATES PATENT OFFICE

LEON LILIENFELD, OF VIENNA, AUSTRIA

## TREATMENT OF FIBROUS MATERIAL

No Drawing. Application filed July 25, 1927, Serial No. 208,402, and in Austria June 9, 1927.

Difficulties are associated with the use of viscose or cellulose solutions as an agent for dressing woven textile materials or sizing yarn, on account of the fact that the fabric or yarn which has been thus treated acquires a stiff, paper-like and cold feel, and moreover its extensibility is rather low. Fabrics which have been dressed by means of viscose have also the disadvantage that the cellulose regenerated from the viscose applied to the fabric frequently undergoes rupture when the material is stretched or pulled, owing to the difference between the coefficients of extensibility of the fabric and the coating, the result being that the coating exhibits numerous minute, or more or less coarse, cracks. Even in textile printing, particularly in pigment printing with viscose, these defects are apparent to an undesirable degree, and the viscose layers printed on the textile have a stiff feel, and in many cases become torn on being stretched, especially when they are not very thin.

This invention relates to a process for treating textile fibrous material (whether in the form of woven fabrics or of yarn) by dressing, sizing, printing, weighting or the like, by means of cellulose in dissolved form (for example viscose or a solution of cellulose in cuprammonia) from which cellulose can be regenerated or precipitated respectively, whereby the foregoing disadvantages are minimized or remedied; the invention includes also the products which can be obtained by the process.

The invention consists in the application of the discovery that the properties of the dressing, sizing, printed layers or the like, which consist of, or contain, cellulose regenerated from soluble derivatives of cellulose, for example from viscose or precipitated from a cellulose solution, for example in cuprammonia, which has been applied to the fibrous material, are improved, especially in respect of feel and extensibility, if the dressing, sizing or coating contains hollow spaces or bubbles dispersed throughout it, or throughout at least a part of it. These hollows or bubbles may be produced by dressing, sizing or otherwise treating the material

with a solution of a soluble modification of cellulose, for example viscose or with a solution of cellulose, containing a quantity of gas or of a substance capable of being caused to evolve a gas by a suitable treatment. Thus textile fabrics or yarns which have been dressed, sized or otherwise treated by means of viscose in accordance with the invention have a soft feel, even when the quantity of the dressing or the like is considerable. The dressing is much lighter, and more downy, and therefore resembles the natural fibre more closely than do the dressings produced in the usual manner from viscose or cellulose solution which is free from gas, or contains but little gas. Fabrics or yarns treated in accordance with the invention have also a warm feel, and owing to the hollows in the dressing, sizing or the like, it is possible to produce even with small proportions of viscose or cellulose solution a very full, rich dressing or sizing. Material treated in accordance with the invention has a good capacity for extension, and fissures or cracks do not occur when the material is pulled or stretched.

The hollow spaces may contain the gas, for example air or carbon dioxide, or the gas may be removed, wholly or in part, from them, for example, by dissolution, or with the aid of an increased or reduced pressure.

In treating fibrous material in accordance with this invention a gas, for example air, hydrogen or nitrogen, may be emulsified in a solution of a soluble modification of cellulose, for example in crude or purified viscose or in a solution of cellulose, for example in cuprammonia, by known methods, such as by injection, blowing, beating, agitation or the like; or the gas may be dissolved in the viscose or other solution with the aid of pressure.

Another method of operating consists in incorporating with the viscose or solution of cellulose a substance, for example an alkali carbonate, which is capable of evolving gas during the treatment for decomposing the viscose or precipitating the cellulose with an agent suitable for the regeneration or precipitation of the viscose respectively.

The viscose containing gas or a substance capable of yielding gas is then applied to or incorporated with a fabric or yarn, by hand, or by means of a suitable machine. In order to cause the viscose or cellulose solution to penetrate more deeply into the fibre, this operation may, if desired, be conducted under reduced pressure, or under a raised pressure. There may be added to the viscose or cellulose solution another coating or sizing agent, for instance, starch, dextrin, albumen or gelatin; a softening agent, for instance, glycerine, soap, Turkey-red oil, glucose, castor oil, or paraffin oil; a filling material, for instance, talc or china clay; a pigment, for instance, zinc white, soot, or powdered mica; or a dyestuff, or any two or more of these substances.

The cellulose may be regenerated from the viscose or precipitated from the cellulose solution in any known manner, by a suitable precipitating bath, or by other means, for instance, by heating, steaming, or merely by allowing the treated material to stand.

If it is desired to expel the gas, for example air, contained in the hollows in order to permit the walls of the hollows to collapse, the gas may be removed for example by boiling with water, or by treatment with water under pressure. If the gas contained in the spaces is carbon dioxide, it may be dissolved partly in the precipitating bath, and partly during the subsequent washing operation.

The following examples illustrate some methods by which the invention may be carried into effect, the parts being by weight:—

*Example 1.*—Air is injected into a viscose, made in any desired manner from matured or non-matured alkali-cellulose containing about 5-7 per cent. of cellulose on analysis, so as to produce an emulsion. A cotton fabric is dressed in known manner in a back-filling machine with the emulsion so produced, and the dressed material is treated, in the wet state or after drying, by any precipitating bath known in the viscose art. The material is then washed, dried and finished in the usual manner.

*Example 2.*—The procedure is as in Example 1, but with the exception that talc is added to the viscose in quantity amounting to about 2-3 parts for each part of cellulose as determined by analysis.

*Example 3.*—100 parts of sulphite-cellulose containing 9-10 per cent. of moisture, or 100 parts of linters containing 7-8 per cent. of moisture are impregnated at 15° C. with 2,000 parts of a solution of caustic soda of 18 per cent. strength. After 3 hours, the soda-cellulose is expressed until its total weight is 300 parts in the case of sulphite-cellulose, or 340 parts in the case of linters, and comminuted in a shredding machine for 2½ to 3 hours. Before the soda-cellulose

has undergone any maturing, 40-60 parts of carbon-disulphide are added, and the mixture is allowed to react for 8 hours at 15-18° C.; at the end of this period any excess of carbon-disulphide which may be present is removed by blowing through a current of air for about 15 minutes, and the cellulose xanthate obtained is dissolved with the aid of a quantity of water, caustic soda and sodium carbonate, such that the solution produced contains 1,220 parts of water, 107 parts of caustic soda and 150 parts of sodium carbonate (reckoned as the anhydrous salt). 75

A suitable cotton fabric is dressed one or more times in a back-filling machine with the viscose produced in the manner just described, after it has been filtered or strained, and in the freshly prepared state, or after it has aged for 48-96 hours at 15° C. The dressed material is then immediately or after having been dried, then introduced into sulphuric acid of 10 per cent. strength, or into any other acid precipitating bath known in the viscose industry, after which it is washed and dried. It will be understood that the material may be desulphurized or bleached in any known manner (for example by means of a solution of sodium sulphide) before or after it has been dried. 80

*Example 4.*—The procedure is as in Example 3, with the exception that the alkali cellulose is allowed to stand for a period of 48-70 hours at room temperature before being treated with carbon disulphide. 85

*Example 5.*—The procedure is as in Example 3 or Example 4, with the exception that talc is added to the viscose, for example, from 10 to 30 parts of the talc per 100 parts of viscose. 100

*Example 6.*—The procedure is as in Example 3, Example 4 or Example 5, with the exception that there is added to the viscose about 1-2 per cent. of its weight of paraffin oil or castor oil. 105

*Example 7.*—The procedure is as in any of the Examples 3-6, with the exception that the viscose has approximately the composition: 100 parts of parent cellulose, 1,260 parts of water, 67 parts of caustic soda, and 150 parts of sodium carbonate (reckoned as the anhydrous salt). 110

*Example 8.*—The procedure is as in any of the Examples 3-6, with the exception that the viscose has approximately the composition: 100 parts of parent cellulose, 1,285 parts of water, 43 parts of caustic soda and 150 parts of sodium carbonate (reckoned as anhydrous salt). 120

The viscose as used in any of Examples 3-8 contains about 6.5 to 6.7 per cent. of cellulose which can be determined by analysis, sodium carbonate being neglected. There may, however, be used a viscose containing a smaller proportion of cellulose, for example, 4-5 per cent. 125

*Example 9.*—100 parts of a viscose containing sodium carbonate as used in any of Examples 3-8 are intimately mixed with 5-8 parts of mica or with 10-15 parts of zinc white. A cotton material is then printed with this mixture in a Rouleaux machine. The further treatment and finishing are conducted in the manner described in the preceding examples.

10 Examples for sizing yarn follow from the foregoing examples.

In carrying out the invention, instead of viscose, there may be used a solution from which cellulose may be precipitated, for example, a solution of cellulose in a thiocyanate solution such as calcium thiocyanate solution, a solution of cellulose in ammoniacal copper oxide solution, a solution of cellulose in an aqueous solution of caustic alkali containing 20 urea, thiourea, or guanidine.

Fabrics and/or yarn dressed or sized respectively, with viscose or any cellulose solution, according to the present process, are under the microscope different from fabrics 25 or yarn filled or sized according to the processes known hitherto with viscose or cellulose solutions. The difference consists in the following: The small cellulose film particles that are on and between the fibres of the fabric 30 or yarn, when produced after the present process, contain hollow spaces and have consequently a spongy structure, whilst the small cellulose film particles formed on and between the fibres of fabrics and yarn that are 35 filled with viscose or cellulose solutions according to the processes known heretofore, do not possess the spongy structure characteristic of fabrics and yarn treated after the present process. Even if fabrics and yarn 40 dressed or sized respectively, after the processes known heretofore, with viscose or any cellulose solution have been after-treated on the so-called breaking machines, the cellulose film particles deposited in or on the fibres 45 show, under the microscope numerous rents, but not a spongy structure characteristic of fabrics and yarn treated according to the present process.

It is to be understood that the term "applying to the fibrous material" includes any manner of application to the fibrous material, whether by manual or mechanical means customary for dressing, sizing, filling, impregnating, coating, weighting or printing 55 a fibrous material, whether in the state of woven fabric or in the state of yarn.

The expression "fibrous material" in the specification and claims includes, wherever the context permits, any spun or woven fibrous material, whether animal or vegetable (for example, flax, linen, hemp, ramie, jute, wool, and particularly cotton) in the form of pure fabrics or in the form of mixed fabrics, or in the form of yarn in skeins, cops or 60 warps.

The expression "cellulose" means in the description and claims: cellulose and its near conversion products, such as cellulose hydrate, hydrocellulose and oxycellulose.

The processes as herein described are 70 claimed in my copending applications Serial Number 305,875, filed September 13, 1928, and Serial Number 393,828, filed September 19, 1929.

The expression "precipitated cellulose" in 75 the following claims includes wherever the context permits, "regenerated cellulose."

Having thus fully described the nature of my said invention and the best means I know for carrying the same into practical 80 effect, I claim:

1. As a new product, fibrous material associated with regenerated cellulose within which are contained hollow spaces containing 85 at least one gas.

2. As a new product fibrous material associated with regenerated cellulose within which are contained hollow spaces containing substantially no gas.

3. Cotton material associated with regenerated cellulose within which are contained hollow spaces, the composite material having an appearance and feel resembling those of pure wool material.

4. As a new product, fibrous material carrying cellulose which, under the microscope, shows numerous hollow spaces.

5. As a new product, fibrous material carrying cellulose which, under the microscope, shows a spongy structure.

6. As a new product, fibrous material carrying precipitated cellulose which, under the microscope, shows numerous hollow spaces.

7. As a new product, fibrous material carrying precipitated cellulose which, under the 105 microscope, shows a spongy structure.

8. As a new product, fibrous material carrying on and between its fibres cellulose which, under the microscope, shows numerous hollow spaces.

9. As a new product, fibrous material carrying on and between its fibres cellulose which, under the microscope, shows a spongy structure.

10. As a new product, fibrous material carrying on and between its fibres precipitated cellulose which, under the microscope, shows numerous hollow spaces.

11. As a new product, fibrous material carrying on and between its fibres precipitated cellulose which, under the microscope, shows a spongy structure.

12. As a new product, fibrous material associated with cellulose films which, under the microscope, show numerous hollow spaces.

13. As a new product, fibrous material associated with cellulose films which, under the microscope, show a spongy structure.

14. As a new product, fibrous material associated with films of precipitated cellulose.

which, under the microscope, show numerous hollow spaces.

15. As a new product, fibrous material associated with films of precipitated cellulose which, under the microscope show a spongy structure.

16. As a new product, fibrous material associated with films of cellulose on and between the fibres, which films, under the microscope, show numerous hollow spaces.

17. As a new product, fibrous material associated with films of cellulose on and between the fibres, which films, under the microscope, show a spongy structure.

18. As a new product, fibrous material associated with films of precipitated cellulose on and between the fibres, which films, under the microscope, show numerous hollow spaces.

19. As a new product, fibrous material associated with films of precipitated cellulose on and between the fibres, which films, under the microscope, show a spongy structure.

In testimony whereof I have signed my name to this specification.

DR. LEON LILIENFELD.